

1

3,053,696

TEXTILE YARN SIZED WITH SODIUM  
CELLULOSE ACETATE SULFATE

George P. Touey and Donald J. Brown, Kingsport, Tenn.,  
assignors to Eastman Kodak Company, Rochester,  
N.Y., a corporation of New Jersey  
No Drawing. Filed Mar. 21, 1960, Ser. No. 16,197  
2 Claims. (Cl. 117—139.5)

This invention relates to a new sizing agent for textile yarns. In particular it relates to a new sizing agent for applying a protective coating to filaments, threads or yarns of cellulose esters during their fabrication into cloth.

In the production of textile materials it is necessary to apply a coating or size to the fibers to protect them from abrasion during the various operations involved in the formation of the cloth. This coating or size must be flexible, tough, and water-soluble. The flexibility and toughness are obvious necessities since the fibers, threads or filaments are twisted and bent in various directions and rub against the shuttle of the loom and against other surfaces during the weaving operation. The coating must be water-soluble so that it can be readily removed from the finished fabric by a simple scouring operation.

In the case of cotton, the most commonly used sizing agent for the thread during the weaving of the cloth is starch. This compound is used extensively in many forms such as the hydrolyzed starches, the dextrans, and the partially etherified or esterified starches containing only a slight amount of the ester or ether substituent group. Examples of the latter are the slightly hydroxyethylated starches and the slightly acetylated starches now commercially available as cotton textile sizes. Also, in the case of cotton such compounds as water-soluble carboxymethyl cellulose, water-soluble hydroxyethyl cellulose and the various water-soluble natural gums (guar gum, gum arabic, sodium alginate, etc.) have been used. Thus, a wide variety of water-soluble polymeric materials have been used with varying degrees of success as sizing agents for cotton textiles.

In the case of the cellulose ester fibers, in particular cellulose acetate, a more difficult sizing problem exists. The conventional cotton sizing agents offer little protection to these threads or filaments during processing into cloth. This is because the applied coatings of such products do not adhere tenaciously to cellulose acetate filaments and are therefore scraped away by abrasion.

Among the many water-soluble polymeric materials which have been recommended as a protective size for cellulose acetate yarn during the weaving operation only a few have ever reached commercial importance. Of these, gelatin and the sodium salt of a maleic acid styrene copolymer are in widespread use. However, gelatin leaves much to be desired as a sizing agent. It is only sparingly soluble in water at room temperatures and dissolves only slowly in water at 140–160° F. Gelatin is also difficult to remove completely from the finished cloth by scouring. This results in residual amounts of the size remaining on the cloth to impair its dyeing characteristics. Finally gelatin, being a natural product, is an excellent source of food for micro-organisms. This must be circumvented by the use of various preservatives in the size make-up solution prior to its application.

Although the styrene-maleic acid copolymer is a synthetic compound which is not easily attacked by micro-organisms, this product also dissolves rather slowly in hot water and is difficultly removed from the cloth after the weaving operation. Moreover this compound, as well as gelatin, imparts a considerable odor to its solutions and to the treated yarn.

2

We have found that sodium cellulose acetate sulfate is an excellent size for cellulose acetate yarn. This substance, which is water-soluble, is a substantially completely esterified mixed ester containing the sodium acid sulfate group ( $-\text{OSO}_3\text{Na}$ ) as the minor ester substituent and the acetoxy radical as the major ester substituent. The preparation of sodium cellulose acetate sulfate has been described in U.S. Patents 2,582,009 and 2,622,079. Its sulfur content can vary between 5% and 13%, and its acetyl content can vary between 10% and 35%. These values represent a cellulose ester with a degree of substitution of 0.4–1.6 sulfate groups and 0.9–2.5 acetyl groups per anhydroglucoside unit. The more important value is the sulfur content of the ester, since this represents the amount of water-solubilizing sulfate groups present in the product. Below a sulfur content of 5% the product is not sufficiently water-soluble to produce a satisfactory sizing solution. Above a sulfur content of 13% the product will not adhere tenaciously to the yarn.

10 This is believed to be due to the low amount of acetyl groups present in a sodium cellulose acetate sulfate which is so highly substituted with respect to the sulfate group. The preferred type of product for our purpose has a sulfur content of 7–11% and an acetyl content of 15–22%.

15 Another factor which must be considered is the viscosity of the water-soluble sodium cellulose acetate sulfate. The method of controlling this viscosity is disclosed in U.S. Patent 2,622,079, column 3. The degradation of the cellulose during the preparation of the mixed

20 ester must be so controlled that the finished product is capable of producing a flowable solution of at least 5% concentration at 25° C. High viscosity types of sodium cellulose acetate sulfate therefore are inoperative because only their very dilute solutions (1–2%) are capable of

25 being free flowing at room temperatures. The high concentrations of such products form gels which will not flow from the size make-up tank and low concentrations (i.e. below 2%) do not produce a sufficient amount of protective film on the fibers to function as a satisfactory size.

30 40 The following examples illustrate our invention without limiting it.

*Example 1.*—A 7% solution of low viscosity type sodium cellulose acetate sulfate was used to size some 75 denier 19 filament cellulose acetate yarn containing one-third of a turn twist per inch. The sized yarn was then checked for abrasion resistance by both the Duplan and the Walker abrasion tests. The Duplan test measures the sized yarn's ability to withstand surface abrasion, while the Walker test measures the sized yarn's ability to withstand flexing. As controls, an unsized yarn and a yarn treated with a commercial cellulose acetate size solution (a styrene-maleic acid, sodium salt size) were also given the Duplan and Walker abrasion tests. Both size solutions contained 6.5% of the sizing agent. The results 45 50 55 were as follows:

|                   | Untreated Control | Yarn Sized With Sodium Cellulose Acetate Sulfate | Yarn Sized With a Commercial Size |
|-------------------|-------------------|--------------------------------------------------|-----------------------------------|
| 60                |                   |                                                  |                                   |
| Duplan value..... | 0                 | 175                                              | 70                                |
| Walker value..... | 70                | 83                                               | 80                                |

These results show that the sodium cellulose acetate sulfate sized yarn had a better abrasion resistance than the same yarn treated with a standard commercial size. The sodium cellulose acetate sulfate used in this experiment had a sulfur content of 9% and an acetyl content of 20%. A 5% solution had a viscosity of 600 c.p.s. at 25° C.

*Example 2.*—The sized cellulose acetate yarns of Exam-

ple 1 were woven into cloth. Both products withstood the abrasion of drop wires, heddle eyes, and reed action during beat up of the filling. There was no evidence of the sizing agent flaking off in either case. However, the cloth with the sodium cellulose acetate sulfate size could be scoured in half the time required for the cloth containing the commercial size.

The Duplan abrasion test is carried out on a Duplan Cohesion Tester, which is a machine designed to test the effectiveness of a slashing solution by testing the cohesion of the sized filament yarn before the warp reaches the loom. Samples of sized yarn under a constant tension are abraded by friction plates moving back and forth on the yarn at a constant rate. The average number of strokes per strand required to separate the filaments in ten strands of yarn are reported as the Duplan value. Forty tests on each sample are considered the standard test. In examining the strands at intervals for open places, an air jet is blown along each strand to assist in detecting openings.

The Walker abrasion test is carried out on a Walker Abrader machine, which is a machine designed to measure the comparative abrasion resistance of strands of yarn. This test applies a controlled amount of localized wear or rubbing between strands of yarn. This rubbing is repeated at regular intervals until breaking occurs, and the number of strokes to failure is taken as a measure of the wearing qualities. The machine is constructed to

test 24 individual specimens of yarn at one time, which allows for variations, and an average of the cycles to failure on 20 specimens is reported as the Walker Abrasion Value. This test is discussed by Tanenhaus in Textile Research J. 17, 281 (1947).

5 We claim:

1. A cellulose acetate textile yarn carrying a sizing of a sodium cellulose acetate sulfate, said sodium cellulose acetate sulfate being a substantially completely esterified mixed cellulose ester containing sodium acid sulfate groups and acetoxy radicals as ester substituents and which has a degree of substitution of 0.4-1.6 sulfate groups and 0.9-2.5 acetyl groups per anhydroglucosidic unit.
- 10 2. A cellulose acetate textile yarn carrying a sizing of sodium cellulose acetate sulfate, said sodium cellulose acetate sulfate being a substantially completely esterified mixed cellulose ester containing sodium acid sulfate groups and acetoxy radicals as ester substituents and which has a sulfur content of from about 7% to 11% and an acetyl content of from about 15% to 22%.

References Cited in the file of this patent

UNITED STATES PATENTS

- |    |           |                                    |
|----|-----------|------------------------------------|
| 25 | 1,950,664 | Dreyfus et al. ----- Mar. 13, 1934 |
|    | 2,134,895 | Seymour et al. ----- Nov. 1, 1938  |
|    | 2,622,079 | Crane ----- Dec. 16, 1952          |